

## UNITED STATES PATENT OFFICE

MILTON O. SCHUR AND ROBERT A. WEBBER, OF BERLIN, NEW HAMPSHIRE, ASSIGNEES  
TO BROWN COMPANY, OF BERLIN, NEW HAMPSHIRE, A CORPORATION OF MAINE

## CELLULOSE DERIVATIVE MANUFACTURE

No Drawing.

Application filed July 20, 1927. Serial No. 207,314.

In the manufacture of cellulose derivatives, it has been the custom to employ various types of cellulosic fibers as a raw material, high grade cotton usually serving where purity and freedom from coloring matter is desired, a wood pulp usually serving where these characteristics are of secondary importance. Even when wood pulp has been refined to an alpha cellulose content approximating 10 that of cotton, it has heretofore failed to yield derivatives of a grade equal to those prepared from high grade cotton, unless special care or treatment is exercised to remove from the fiber certain impurities which survive the refining treatment to a very slight degree but which exert a powerful and highly undesirable coloring effect in the preparation of cellulose derivatives. 15 If wood pulp, for example, is examined closely, it will be observed that it consists of units of varying fiber lengths, some being considerably above and some considerably below the average fiber length of the pulp as a whole. A considerable portion of the pulp 20 exists in the form of fibrillæ, short and broken fiber, and colloidal cellulose. We have observed that pulp in finely divided or colloidal condition and hereinafter designated as "fines" has the property of adsorbing impurities of various kinds, tests showing that this 25 portion of a pulp contains far more impurities than the rest of the pulp. The fines are rich in resins, waxes, fats, and other impurities extractable by organic solvents, sometimes containing over 7% of substance soluble 30 in hot carbon tetrachloride. They are also high in ash content. The proportion and composition of fines in a given pulp depend upon the particular conditions and process of 35 fiber liberation, and also upon the character of the wood from which the pulp was derived. They are, however, always darker in color and more resistant to whitening with bleach than the rest of the pulp. They are, 40 moreover, so sensitive to heat that they yellow when made into a sheet and dried on a steam drum under temperature conditions simulating pulp and paper mill practice. Owing to the fact that the impurities along 45 the alpha cellulose are reacted upon, a cellulose

derivative prepared therefrom is dark in color and comparatively unstable.

In accordance with our process, these fines are removed from the pulp before it is converted into cellulose derivatives, as we have 55 found that the quality of derivatives preparable from the resulting pulp is greatly superior to those preparable from the original pulp. The removal of fines is advantageous 60 in the case of the various wood pulps and other cellulosic materials employed in producing cellulose derivatives, and is especially advantageous where wood pulp is being refined to a high alpha cellulose content, as in such case the resulting pulp is substantially equal 65 to high grade cotton for the production of cellulose derivatives. Ordinarily, the impurities associated with the finest content of a pulp degrade it to some extent, but when 70 fines are removed these impurities are also removed, so that the quality of the stock and the characteristics of the cellulose derivatives are vastly improved.

The removal of the fines may be effected 75 at any suitable stage in the chemical processing of the pulp intended to condition it for derivative manufacture. Preferably, however, the fines are removed from the unbleached pulp in order to avoid their chemical processing. Processing is thus effected 80 only upon the valuable portion of the pulp, thereby enabling a saving of the chemicals. For instance, if pulp, e. g., sulphite, is only to be bleached prior to conversion into cellulose derivatives, a removal of the fines may 85 be accomplished advantageously just before the pulp is bleached, so as to enable easy and rapid bleaching to a bright, practically pure white color with a minimum quantity of bleach. Where the pulp is to be refined to a high alpha cellulose content by a series of 90 chemical treatments, for instance by a series which includes chlorination of the unbleached pulp, followed by alkaline digestion and by bleaching, a removal of the fines may be effected before or after any one of the chemical treatments, although in such case, too, it is preferable to accomplish this 95 removal before the first chemical treatment, 100

as a saving of chemicals in all the treatments may be realized.

The removal of the fines from the pulp may be effected as disclosed in application, Serial No. 755,730, filed December 13, 1924, by George A. Richter and Elwood Ebie. In this process, wood pulp is washed against fine mesh wire, for instance, 50-mesh Fourdrinier wire, or against thin plates provided with perforations of, say, 0.02 inches in diameter. The washing may be effected as by repeatedly diluting the pulp with fresh filtered water to a consistency of about 1%, and then thickening the pulp by causing it to flow against the screens or plates arranged in an inclined position. Such washing results in the fines passing through the wire or plates, and the perfect fiber remaining on the screens or plates. Where unbleached wood pulp is so treated, the proportion of material passing through the screens or plates may be from 4% to 25% of the weight of the original pulp. The perfect fiber may then be chemically processed as previously described, to effect its refinement to a high alpha cellulose content. The refined product is stable toward heat and light, and yields cellulose derivatives, for example, nitrocellulose, as stable and free from coloring matter as those prepared from high grade cotton. When it is nitrated, little color is imparted to the mixed nitrating acids, so that after nitration they may be fortified and reused for effecting the nitration of other pulp.

If desired, the long fibers may be separated from the pulp, the method employed, for instance, being that described in application, Serial No. 206,477, filed July 18, 1927, by Robert A. Webber. This method involves passing edge-presenting members capable of picking up the long fibers, through the pulp suspension, and then washing off and recovering the long fibers picked up from the edge-presenting members. The long fibers thus picked up are eminently suitable for the manufacture of pure and stable derivatives, as hereinbefore described.

The fines obtained in our process may be bleached or refined and bleached, and marketed for the manufacture of inexpensive papers or derivatives. While unsuitable for the manufacture of high grade papers because of their short fiber length, they are quite suitable for the preparation of derivatives when high quality is not desired. This is particularly true where these fines have been refined along with the rest of the pulp and where color or high degree of purity in the derivatives is of secondary consideration, low price being more important. Thus, such fines, particularly when refined, are suitable for the preparation of nitrocelluloses to be used in the manufacture of cheap celluloid toys, advertising novelties, and the

like. In other words, they offer an attractive source of raw material, where low price is an important factor. For the preparation of high grade cellulose derivatives where quality is of paramount consideration, however, wood fiber from which the fines have been removed is more suitable.

By the process of the present invention, it is possible to enhance greatly the value not only of derivatives prepared from wood fiber, but also of derivatives prepared from cellulose fiber of other origins. Thus, we have even realized a worth-while improvement in the color of derivatives, particularly the products of nitration, when the fines were removed from cotton linters.

We herein do not claim the subject matter of application Serial No. 202,454, filed June 29, 1927, by George A. Richter and Milton O. Schur, which discloses a process of freeing cellulose pulp from resinous impurities, or the product resulting from such process; nor do we herein claim the subject matter of application Serial No. 210,998, filed August 5, 1927, by George A. Richter and Milton O. Schur, and issued October 1, 1929, as Patent No. 1,729,629, which discloses a process of separating out the fraction containing fine, short, and broken fibers from cellulose pulp, removing resinous and other impurities from the fraction separated out, and converting the deresinified fraction into cellulose derivatives.

Having thus described our invention, it should be obvious to those skilled in the art that it is subject to change and modification without departing from its spirit or scope as defined in the appended claims.

What we claim is:

1. A process which comprises separating the finely divided and colloidal cellulose together with associated impurities from the longer fibers in fibrous cellulosic materials, then converting the long fibers into cellulose derivatives.

2. The process which comprises converting into cellulose derivatives high alpha cellulose pulp freed from the finely divided and colloidal cellulose together with associated impurities.

3. A process which comprises removing finely divided and colloidal cellulose from wood pulp, and then converting the rest of the pulp into cellulose derivatives.

4. A process which comprises removing finely divided and colloidal cellulose from wood pulp, and then nitrating the remaining pulp.

5. A process which comprises removing finely divided and colloidal cellulose from unbleached wood pulp, bleaching the remaining pulp, and converting the bleached pulp into a cellulose derivative.

6. A process which comprises removing finely divided and colloidal cellulose from un-

bleached wood pulp, chemically refining the remaining pulp to high alpha cellulose content, and converting it into a cellulose derivative.

5 7. A process which comprises removing finely divided and colloidal cellulose from unbleached wood pulp, chlorinating, alkaline digesting, and bleaching the remaining pulp, and converting it into a cellulose derivative.

10 In testimony whereof we have affixed our signatures.

MILTON O. SCHUR.  
ROBERT A. WEBBER.

15

20

25

30

35

40

45

50

55

60

65